

## UNITED STATES PATENT OFFICE.

ALEX BROOKING DAVIS, OF CINCINNATI, OHIO, ASSIGNOR TO A. B. DICK COMPANY, OF CHICAGO, ILLINOIS, A CORPORATION OF ILLINOIS.

## MANUFACTURE OF STENCIL SHEETS.

No Drawing. Original application filed February 5, 1926, Serial No. 86,343. Divided and this application filed August 5, 1926. Serial No. 127,486.

Reference is hereby made to an application filed by me February 5, 1926, for stencil sheets and coating masses therefor, Serial No. 86,343, of which this application is a 5 division.

The present invention relates particularly to stencil sheets made by depositing upon a porous base sheet, such as Japanese yoshino paper, a homogeneous type and stylus im- 10 pressible film. Many types of stencils of this character have already been made, either by drawing the Japanese yoshino paper through molten coating masses such as those which may be compounded from 15 waxes, gums, etc., or by depositing upon the yoshino sheet homogeneous films by drawing the sheets through solutions of various substances and allowing the volatile solvent to evaporate. Other processes than the two 20 above stated have been used for depositing the film upon the yoshino paper, but all forms of stencil sheets so far produced have possessed certain disadvantages, such as lack of strength and working qualities, deteriora- 25 tion on standing, or the easy breaking of the film unless the paper be handled with care.

The object of this invention is to provide a new stencil coating mass which eliminates many of the usual difficulties of production, 30 and to provide stencil sheets possessing marked advantages as to toughness, clean- 35 ness of impression, working qualities, and which keep without deterioration when stored for long periods. Other objects of my invention will be in part obvious and in part pointed out hereinafter.

In carrying out the invention, I may proceed as follows:

Acetone-soluble cellulose acetate such as 40 is normally used for the production of artificial silk is dissolved in acetone to a 10% solution by weight. According to the character of the cotton used in the production of the cellulose acetate and the method of 45 acetylation, the viscosity of the cellulose acetate solution varies over wide limits, and while all types of the cellulose acetate which I have been able to obtain will give a stencil sheet, I prefer to use that grade which may 50 be called "medium viscosity." Into a suitable vessel there is placed 120 parts by

weight of this 10% cellulose acetate solution in acetone. There is now added 200 parts by weight of acetone. Into this mass there is now stirred 100 parts by weight of mono 55 benzoyl butyl tartrate, in which has been dissolved 20 parts by weight of chlorinated naphthalene, and for this material I prefer the solid chlor derivatives consisting mainly of the tetra, penta and hexa chlor com- 60 pounds. The mono benzoyl butyl tartrate, which I believe to be a hitherto unused and unknown substance, is made preferably by reacting upon the dinormal butyl ester of tartaric acid with benzoyl chloride by heat- 65 ing the two substances together until hydrochloric acid ceases to be given off and the resulting oil reacts practically neutral.

Into the resulting mass there is now stirred as a pigment to lend opacity 10 parts by 70 weight of zinc oxide which has been previously ground in 10 parts by weight of butyl tartrate. The mass is now stirred thoroughly and forms a homogeneous lac- 75 quer-like body, from which stencils may be produced by drawing sheets of Japanese yoshino paper, or other suitable porous, fibrous base sheets, through or over and removing the excess by pulling the sheets over a wire. The resulting stencil sheets 80 are then hung up on racks to allow the volatile solvent, principally acetone, to evaporate. This evaporation takes place very rapidly, and in a comparatively short period of time the sheets may be removed to be 85 mounted upon proper backing sheets, ready for use in the typewriter or with the stylus for the production of stencils to be used on duplicating machines. Such sheets are semi-opaque, nearly white in color, and 90 possess a marked degree of toughness. The film does not break easily or crack, and the stencils which result from the use of the typewriter or stylus give very superior results in number of copies, and the excellence 95 of the work which they produce is easily evident upon examining the copies, particularly when a high grade ink best suited for the work is used on the duplicating machine.

An alternative formula which gives re- 100 sults of a highly satisfactory and similar

|                                                                       |      |
|-----------------------------------------------------------------------|------|
| character is as follows, all parts being by weight:                   |      |
| Cellulose acetate basis dry-----                                      | 225  |
| Acetone-----                                                          | 4000 |
| 5 Mono benzoyl butyl tartrate-----                                    | 1125 |
| Zinc oxide ground in mono benzoyl butyl tartrate 50-50 by weight----- | 300  |
| Diamyl phthalate-----                                                 | 375  |
| 10 Chlorinated naphthalene (as above described)-----                  | 225  |
| Castor oil-----                                                       | 60   |

It is obvious from the above formula that certain constituents may be regarded as basic and essential, particularly the cellulose acetate, and color must be lent by a pigment or a dyestuff, but the remaining ingredients may be replaced or substituted by other materials of slightly different composition. For instance, the mono benzoyl butyl tartrate may be replaced by other derivatives of butyl tartrate in which one or more of the hydroxyls of the tartaric acid radical have been combined with some other acid; thus, I have found mono acetyl butyl tartrate satisfactory. The chlorinated naphthalene may be replaced by other hydrocarbons or halogenated hydrocarbons, particularly those of the anthracene series, such as anthracene itself and carbazol. The diamyl phthalate in the second formula may be exchanged for butyl phthalate and the castor oil for other vegetable or animal oils of similar character and properties.

35 As a further alternative formula, the following will serve:

To 75 grams of 10% solution of cellulose acetate in acetone, there is added 25 grams of 33% solution of starch acetate in acetone. 40 There is now stirred in 70 grams of mono benzoyl butyl tartrate and 15 grams of a halogenated aromatic hydrocarbon, such as hexachlor naphthalene. A quantity of coloring matter or pigment may be added to 45 give color to the mass.

In the above formula, the application of the invention is broadened by the use as a constituent of a second carbohydrate ester in the form of starch acetate, showing the broad application of the invention to carbohydrate esters in general and particularly for the production of coating masses for the manufacture of stencil sheets.

The mono benzoyl butyl tartrate used primarily in the description of this invention is only a representative of a group of substances which may be classed as acid substituted derivatives of hydroxy acid esters, a large number of which I have found to 55 possess properties similar to the mono benzoyl butyl tartrate and upon which I have a group patent pending at the present time. Acetyl amyl tartrate, benzoyl amyl salicylate, benzoyl ethyl lactate, and kindred substances, all of which may be classed as acid

substituted hydroxy acid esters, fall within the scope of this invention as representative of substances which may be used in place of the mono benzoyl butyl tartrate, and I therefore, do not restrict myself to any particular representative of this group of substances as a primary modifying agent in formulæ of the character given above.

50 Stencils produced from this coating mass are capable of yielding large numbers of copies when used with the usual forms of duplicating machines, and the impressions which they give are clean of line and sharply defined; in fact, the number of impressions which can be obtained from these stencils, even on power driven duplicating machines, is far greater than the requirements of the average user for any individual stencil.

55 Now having described my invention, what I claim is:—

1. A type-impressible stencil sheet coating including cellulose acetate and benzoyl butyl tartrate.
2. A type-impressible stencil sheet coating including cellulose acetate and mono benzoyl butyl tartrate.
3. A type-impressible stencil sheet coating including cellulose acetate and an ester of tartaric acid in which at least one hydroxyl has been combined with an acid radical.
4. A type-impressible stencil sheet coating including cellulose acetate and an acid substituted dialkyl ester of tartaric acid.
5. A type-impressible stencil sheet coating including cellulose acetate and an acid substituted dialkyl ester of tartaric acid and a halogenated hydrocarbon.
6. A type-impressible stencil sheet coating including cellulose acetate, an acid substituted dialkyl ester of tartaric acid and a hydrocarbon.
7. A type-impressible stencil sheet coating including cellulose acetate, a tartaric acid ester, an acid substituted dialkyl ester of tartaric acid and an ester of phthalic acid.
8. A type-impressible stencil sheet coating including cellulose acetate, a tartaric acid ester, an acid substituted dialkyl ester of tartaric acid, an ester of phthalic acid and a halogenated hydrocarbon.
9. A type-impressible stencil sheet coating including cellulose acetate, a tartaric acid ester, an acid substituted dialkyl ester of tartaric acid, an ester of phthalic acid and a hydrocarbon.
10. A type-impressible stencil sheet coating including cellulose acetate, an acid substituted tartaric ester and a vegetable oil.
11. The process of manufacturing a type-impressible stencil sheet for use with duplicating machines, which consists of depositing upon a porous base sheet a homogeneous film including cellulose acetate and benzoyl butyl tartrate by means of a volatile solvent.
12. The process of manufacturing a type-

impressible stencil sheet for use with duplicating machines, which consists of depositing upon a porous base sheet a homogeneous film including cellulose acetate and mono 5 benzoyl butyl tartrate.

13. The process of manufacturing a type-impressible stencil sheet for use with duplicating machines, which consists of depositing upon a porous base sheet a homogeneous 10 film including cellulose acetate and an ester of tartaric acid in which at least one hydroxyl has been combined with an acid radical.

14. The process of manufacturing a type-impressible stencil sheet for use with duplicating machines, which consists of depositing upon a porous base sheet a homogeneous film including cellulose acetate and an acid 15 substituted dialkyl ester of tartaric acid.

15. The process of manufacturing a type-impressible stencil sheet for use with duplicating machines, which consists of depositing upon a porous base sheet a homogeneous film including cellulose acetate, an acid substituted dialkyl ester of tartaric acid and a 20 halogenated hydrocarbon.

16. The process of manufacturing a type-impressible stencil sheet for use with duplicating machines, which consists of depositing 25 upon a porous base sheet a homogeneous film including cellulose acetate, an acid substituted dialkyl ester of tartaric acid and a hydrocarbon.

17. The process of manufacturing a type-impressible stencil sheet for use with duplicating machines, which consists of depositing 30 upon a porous base sheet a homogeneous film including cellulose acetate, a tartaric acid ester, an acid substituted dialkyl ester of tartaric acid and an ester of phthalic acid.

18. The process of manufacturing a type-impressible stencil sheet for use with dupli-

cating machines, which consists of depositing upon a porous base sheet a homogeneous 45 film including cellulose acetate, a tartaric acid ester, an acid substituted dialkyl ester of tartaric acid and a halogenated hydrocarbon. 50

19. The process of manufacturing a type-impressible stencil sheet for use with duplicating machines, which consists of depositing upon a porous base sheet a homogeneous film including cellulose acetate, a tartaric 55 acid ester, an acid substituted dialkyl ester of tartaric acid, an ester of phthalic acid and a hydrocarbon.

20. The process of manufacturing a type-impressible stencil sheet for use with duplicating machines, which consists of depositing upon a porous base sheet a homogeneous film including cellulose acetate, an acid substituted tartaric ester and a vegetable oil. 60

21. A type-impressible stencil sheet coating including an acid substituted hydroxy acid ester and a carbohydrate ester. 65

22. A type-impressible stencil sheet coating including a carbohydrate ester and a hydroxy acid ester at least one hydroxyl of 70 which has been combined with an acid group.

23. A type-impressible stencil sheet including in its coating composition a carbohydrate ester and the reaction product of an 75 organic acid halogen upon a hydroxy acid ester.

24. A type-impressible stencil sheet including in its coating composition cellulose acetate, starch acetate, an acid substituted 80 hydroxy acid ester and a substance with lubricating power.

This specification signed this 26th day of July, 1926.

ALEX BROOKING DAVIS.